# EUROPEAN PATENT APPLICATION

(11) **EP 0 316 541 A1**
(43) Date of publication of application: **24.05.1989**
(21) Application number: 88115387.8
(22) Date of filing: 20.09.1988
(51) Int. Cl.: B22F 3/22, B28B 1/26, B28B 13/02

(54) **Method for casting powder into a compact and apparatus therefor**

(30) Priority: 13.11.1987 JP 287130/87
(71) Applicant: NKK CORPORATION, Tokyo (JP)
(72) Inventor: Nishio, Hiroaki c/o Pat. Lic. & Qual. Stand. Dept., Chiyoda-ku Tokyo (JP); Kawashima, Takeshi c/o Pat. Lic. & Qual. Stand., Chiyoda-ku Tokyo (JP)
(74) Representative: Füchsle, Klaus, Dipl.-Ing.

(57) **Abstract**

A method for casting powder into a compact comprises: charging material powder into a slurry vessel (1) to prepare slurry of the material powder; removing air contained in the slurry by reducing an inside pressure of the slurry vessel; casting the slurry into a mould (11) by applying a pressure to the slurry as the inside pressure is kept at the reduced pressure; and cooling the slurry through the mould (11) to solidify the slurry into a compact and thereafter demolding the mould (11). Further an apparatus for the method comprises: a slurry vessel (1) capable of preparing slurry of material powder and of keeping an inside pressure of the slurry vessel (1) at a reduced pressure; means for reducing the inside pressure; a mould (11) having a cooling conduit tube in the mould (11); and a slurry pump (7) for transferring the slurry from the slurry vessel (1) to the mould (11).

## Description

The present invention relates to a method for casting metallic or ceramic powder into a compact and an apparatus therefor, and more particularly to a method for casting the metallic or ceramic powder, wherein such powder is made into slurry and the slurry is cast by application of pressure thereto and an apparatus for the method.

As a prior art method of casting a metallic or ceramic powder, in particular for forming a complicatedly-shaped compact, Pertsman type casting method is known (Casting of Fine Ceramics and Organic Material published by CMC Co., Ltd. August 26, in 1985). This method is applicable to casting a mixture of various kinds of powder, for example, metallic powder such as 2%Ni-98%Fe and SUS316, ceramic powder such as alumina, silicon-carbide, zirconia and ferrite and mix powder of metal and ceramics such as tungsten carbide-cobalt and titanium carbide-nickel.

The outline of the casting method is to add a binder mainly composed of paraffin to such powder as the aforementioned to form slurry, and to cast the slurry in a mold by application of pressure to obtain a compact. In stead of the paraffin ordinarily used, substance such as stearyl alcohol and stearic acid having low viscosity at melting and solidifying easily by cooling can be used. Furthermore, sometimes oleic acid, bees wax or the like is also added to improve plasticity of the slurry.

Now, referring specifically to Fig. 2 of the drawing, prior art, Fig. 2 is an explanatory view schematically illustrating an apparatus of the Pertsman type casting. This apparatus comprises stirrer 3, slurry vessel 1 wherein material powder and binder such as paraffin are mixed to become a homogeneous slurry and store the slurry temporarily, a vacuum pump 5 reducing an inside pressure of slurry vessel 1, air compressor 20 increasing the inside pressure of slurry vessel 1 and mold 11 having cylinder 13. Slurry vessel 1 and pipes connecting various devices are prepared so as to be heated from the outside, as required.

To form a compact by means of the apparatus thus constituted, material powder such as metallic or ceramic powder is put into slurry vessel 1 through inlet 2 of slurry vessel 1 together with paraffin, bees wax and the like and stirred by stirrer 3 to prepare slurry. Next, vacuum pump 5 is started to work and reduce an inside pressure of the vessel to remove air contained in the slurry. When the removal of the air is completed, the operation of the stirrer and vacuum pump 5 are stopped. And then, air compressor 20 is started to work and a pressure is applied to the slurry in the vessel. The slurry with the increased pressure is charged into mold 11 provided with an air cylinder 13 for fixing the mold so as to be stable provided, however, that the mold was cooled by means of passing cooling water 12 in advance of the charging. Then, after the slurry in the mold has been formed into a compact, air compressor 20 is stopped and the increased inside pressure is returned to a level of atmospheric pressure. Subsequently, the cylinder is taken off and the mold is demolded. Thus, the compact is taken out.

The prior art method, however, has a drawback in that the density of a produced compact is by 2-5% lower than the theoretical density (a value computed from ratio of material powder and binder and from each true density of the two) due to air being included in the slurry through casting step, and pores corresponding to the drop of the product density are produced, thereby the quality of the product is degraded. This is because due to the application of the pressure to the slurry in vessel 1 at the time of casting, the free surface of the slurry is brought into contact with the pressure-increased air and this air goes again into the slurry, although air contained in the slurry is firstly removed by means of reducing the inside pressure of vessel 1. Furthermore, the prior art method is disadvantageous in that the surface of the slurry above an outlet of the vessel forms a concavity. This is because the viscosity of the slurry at the time of casting is so high that the surface of the slurry does not go down equally as the slurry is discharged and, depending on the terms of casting such as viscosity and casting speed, the part of the slurry contacting with the wall of vessel 1 and stirrer 3 goes down slower and, as a result, the slurry existing just above the outlet of the vessel goes down comparatively faster. Since the concavity of the slurry becomes exceedingly large depending on condition of the operation, slurry existing around the concavity portion is collapsed and a large amount of air is often sucked into the slurry. In such case, it happens that air contained in the slurry being cast bursts out through gaps of the mold, or the air is solely sent into the mold and bursts out continuously in spite of the slurry remaining in the vessel. This results in making it impossible to cast the slurry into a compact.

The object of the present invention is to provide a method for casting powder into a compact wherein the casting is carried out continuously and stably without not only inclusion of air in slurry but also suction of a large amount of air into the slurry at the time of casting the slurry.

To attain the object of the invention, in accordance with the present invention, a method for casting powder into a compact comprises:
charging material powder into a slury vessel to prepare slurry of the material powder;
removing air contained in the slurry by reducing an inside pressure of the slurry vessel;
casting the slurry into a mold by applying a pressure to the slurry as the inside pressure is kept at the reduced pressure; and
cooling the slury through the mold to solidify the slurry into a compact and thereafter demolding the mold.

Furthermore, to carry out the method as defined in the foregoing, in accordance with the present invention, an apparatus comprises:
a slurry vessel capable of preparing slurry of material powder and of keeping an inside pressure of the slurry vessel at a reduced pressure;
means for reducing the inside pressure;
a mold having a cooling conduit tube in the mold;
and
a slurry pump for transferring the slurry from the slurry vessel to the mold.

The object and other objects and advantages will become clear from the detailed description to follow, taken in conjunction with the appended drawings.
Fig. 1 is an explanatory view illustrating schematically an apparatus for casting powder into a compact according to the present invention; and
Fig. 2 is an explanatory view illustrating schematically a prior art apparatus for casting powder into a compact.

Referring specifically to the drawings, a preferred embodiment will now be described. Fig. 1 shows schematically an explanatory view of an apparatus for casting powder into a compact. Referential numeral 1 denotes a slurry vessel having material inlet 2 at the upper portion thereof and stirrer 3 and the slurry vessel is capable of keeping an inside pressure of the slurry being reduced. Exhausting pipe 4 is fitted to the upper portion of the slurry vessel and is connected to vacuum pump 5 as means for reducing the inside pressure of the slurry vessel. In this embodiment a rotary pump is used for the vacuum pump. At the bottom of the slurry vessel there is provided lead pipe 6 connecting to slurry pump 7. From exhausting outlet of the slurry pump, pipe 8 extends and reaches mold 11 through valve 9. Mold 11 is made from material having characteristic of not absorbing liquid and is placed fixedly on support table 10 by using pressure of air cylinders 13 (one air cylinder is shown for simplification). Mold 11 is pressed vertically or horizontally or both vertically and horizontally by air cylinder 13 to prevent the mold from expanding its shape due to an inside pressure of the slurry which has been given by slurry pump 7.

Before reaching valve 9 from slurry pump 7, pipe 8 branches out into branch pipe 14. Due to pipe 14 being arranged, the slurry sent out of slurry vessel 1 can be returned to slurry vessel 1 through pressure control valve 15 and be recirculated. At the same time, by means of pressure control valve 15, a pressure for casting the slurry in mold 11 can be controlled.

It should be noted that because the temperature of the slurry is required to be kept at the melting point or more of a binder used, heaters 16 are attached to slurry vessel 1, pipe 8 and branch pipe 14 to heat each of them up to such a temperature as required. The slurry pump used for the apparatus of the present invention is a forced pump which can be any one of a tube pump, an eccentric screw pump and a diaphragm pump.

Secondly, an embodiment of a method using the apparatus of the present invention now will be described. Material powder such as metallic or ceramic powder, a binder together and an additive are charged into slurry vessel 1 through inlet 2 of the slurry vessel and then, stirrer 3 is operated. Vacuum pump 5 as means for reducing an inside pressure of the slurry vessel is started to work. While by means of vacuum pump 5 the inside pressure of the slurry vessel is reduced and air therein is removed, a heaters 16 is operated to form those charged materials into slurry and the slurry is heated up to a predetermined temperature. After the slurry is elevated to the predetermined temperature, the slurry continues to be stirred by stirrer 3 for 3 hours. Then, slurry pump 7 begins to be operated and the slurry is circulated through pipe 8 and branch pipe 14. During the circulation, the stirring by stirrer 3 is continued at a reduced pressure for about an hour to remove air contained in the slurry by the operation of vaccum pump 5. As a result, the removal of air is effectively carried out.

Subsequently, mold 11 is placed on support table 10 and air cylinder 13 is arranged to work. Then, the pressure of the air cylinder is applied to the mold and the mold is fixedly and stably set on the support table not so as for the mold to expand and, cooling water 12 is passed through a condit tube in the mold. Pressure control valve 15 is also arranged to set a predetermined pressure value for the slurry to be cast. Now, valve 9 is opened and then, the slurry is transferred into mold 11 and is cast therein. After a predetermined time of the casting, the valve is closed. And then, the pressure of air cylinder 13 is released, the mold is demolded and a compact is taken out.

In the mentioned step of casting the slurry, after reducing an inside pressure of slurry vessel 1 and removing air therein, the slurry is transferred to mold 11 as the inside of the slurry vessel is kept at such reduced pressure and the slurry is cast into a compact in the mold. Therefore, air is not mixed into the compact. The inside pressure to be reduced at casting i.e. the atomospheric pressure of the slurry vessel is of 100 to 10-3 Torr, thereby the compact not including air being obtained. If the inside pressure of the slurry vessel is more than 100 Torr, it is difficult to prevent air from being mixed again into the slurry during the casting process. Of course, the lower limit of the reduced pressure is dependent on conditions such as a kind of binders and concentration of slurry, but in any event, so long as the pressure is chosen in the range of not less than 10⁻³ Torr, the prevention can be attained. To make the pressure less than 10⁻³ Torr, a machinery pump with high capability of reducing pressure, for example, a diffusion pump must be used. This results in raising cost. In addition, a slurry pump used in the apparatus of the present invention, as means for transferring the slurry to mold 11, is recommended to be a forced pump which is hard to allow foreign matters such as gas and oil put into the mold together with the slurry at the time of the transfer thereof.

### Example

In this example, mixed ceramic powder of silicon nitride was cast by using an apparatus having a constitution as shown in Fig. 1 and a flat plate with the size of 70mm x 100mm x 10mm was produced.

1,000g of mixed powdelr consisting of Si₃N₄ Y₂O₃ and Al₂O₃ having the mixed r;tio as shown in Table 1 together with 157g of paraffin and 25g of bees wax was charged into slurry vessel 1 and slurry of those charged materials was prepared according to the steps as described in the detailed description. When the inside pressure of the slurry vessel was reduced to remove air therein, the temperature of the slurry was 92°C and the inside pressure was 0.05 Torr. The slurry was cast at the pressure of 3kg/cm² in mold 11 by slurry pump 7 and a compact was thus obtained. The density of the compact was equal to the theoretical density as shown in Table 2.

In comparison with the example of the present invention, the same material with the example was cast by using a prior art apparatus having a constitution as shown in Fig. 2 and a controller of a flat plate compact having the same size with that of the example was produced. The reduction of the inside pressure of slurry vessel 1 and the removal of air in the slurry vessel was carried out on the same condition with the example. The temperature of the slurry was 92°C and the inside pressure was 0.05 Torr as well. And then, air compressor 20 was started to work and tle inside pressure was increased to 3 kg/cm² to cast the slurry into the controller in mold 11. The density of the controller was 96% of the theoretical density as shown in Table 2. When the slurry was reduced to about a half of the initial amount in the slurry vessel to produced compacts as controllers, air began to be sucked into the slurry and thereafter this phenomenon of the suction often occurred. The casting was instable and the operation was not easy.

As described in the detailed description, according to the apparatus and the method of the present invention, a compact without pores can be obtained. This is because the slurry is sent to mold 11 as kept at a reduced pressure in slurry vessel 1 and air is not sucked into the slurry. In addition, a continuous and stable casting operation can be attained. This is because the inside of the slurry vessel is kept at the reduced pressure and no air is sucked into the slurry, even if the part of the slurry existing justs above an outlet exclusively goes down fast in the slurry vessel and the surface of the slurry forms a concavity when the amount of the slurry in the slurry vessel decreases in the casting process.

## Claims

1. A method for casting powder into a compact which comprises:
charging material powder into a slurry vessel to prepare slurry of the material powder;
removing air contained in the slurry by reducing an inside pressure of the slurry vessel;
casting the slurry into a mould by applying a pressure to the slurry as the inside pressure is kept at the reduced pressure, and
cooling the slurry through the mould to solidify the slurry into a compact and thereafter demoulding the mould.

2. The method of claim 1, characterized in that the reducing an inside pressure includes reducing the inside pressure to 100 to 10⁻³ Torr.

3. The method of claim 1 or 2, characterized in that the casting the slurry into a mould includes casting the slurry by controlling a pressure given to the slurry.

4. The method of claim 1, 2 or 3, characterized in that the casting the slurry into a mould includes casting the slurry through a pipe connecting a slurry pump and the mould.

5. The method of claim 4, characterized in that the casting the slurry into a mould includes casting the slurry by controlling a pressure of the slurry to be supplied to the mould by means of returning the slurry to the slurry vessel through a branch pipe with a pressure control valve branching out from the pipe.

6. The method of any one of claims 1 to 5, characterized in that the removing air contained in the slurry includes removing the air as the slurry is being circulated through a lead pipe connecting the slurry vessel and a slurry pump, a pipe connecting the slurry pump and the mould and a branch pipe branching out from the pipe and reaching the slurry vessel.

7. An apparatus for casting powder into a compact which comprises:
a slurry vessel (1) capable of preparing slurry of material powder and of keeping an inside pressure of the slurry vessel (1) at a reduced pressure;
means for reducing the inside pressure; and a mould (11) having a cooling conduit tube in the mould,
characterized by a slurry pump (7) for transferring the slurry from the slurry vessel (1) to the mould.

8. The apparatus of claim 7, characterized in that the slurry pump (7) for transferring the slurry includes a forced pump.

9. The apparatus of claim 8, characterized in that the forced pump includes any one selected from a tube pump, an eccentric screw pump and a diaphragm pump.

10. The apparatus of claim 7, 8 or 9, characterized in that the slurry vessel (1) includes having a heater (16).

11. The apparatus of any one of claims 7 to 10, characterized by further comprising a pipe (8) and a branch pipe (14), the pipe (8) connecting the slurry pump (7) and the mould, and the branch pipe (14) branching out from the pipe (8) and reaching the slurry vessel (1).

12. The apparatus of claim 11, characterized in that the pipe (8) and the branch pipe (14) includes having a heater (16) for each of the pipe (8) and the branch pipe (14).

13. The apparatus of claim 11 or 12, characterized in that wherein the branch pipe (14) includes having a pressure control valve (15).
